



US006184772B1

(12) **United States Patent**  
Kawase et al.

(10) **Patent No.:** US 6,184,772 B1  
(45) **Date of Patent:** \*Feb. 6, 2001

(54) **CHIP THERMISTORS**

5,534,843 \* 7/1996 Tsunoda et al. .... 338/22 R

(75) Inventors: **Masahiko Kawase; Norimitsu Kitoh,**  
both of Shiga (JP)

(73) Assignee: **Murata Manufacturing Co., Ltd.,**  
Kyoto (JP)

(\*) Notice: This patent issued on a continued prosecution application filed under 37 CFR 1.53(d), and is subject to the twenty year patent term provisions of 35 U.S.C. 154(a)(2).

Under 35 U.S.C. 154(b), the term of this patent shall be extended for 0 days.

(21) Appl. No.: **09/124,194**

(22) Filed: **Jul. 28, 1998**

(30) **Foreign Application Priority Data**

Aug. 7, 1997 (JP) ..... 9-213413

(51) **Int. Cl. 7** ..... H01C 7/10; H01C 7/13

(52) **U.S. Cl.** ..... 338/22 R; 338/225 D;  
338/204

(58) **Field of Search** ..... 338/22 R, 225 D,  
338/101, 204, 334

(56) **References Cited**

**U.S. PATENT DOCUMENTS**

4,685,203 \* 8/1987 Takada et al. ..... 29/620

**FOREIGN PATENT DOCUMENTS**

1-289201 \* 11/1989 (JP) .  
6-302406 4/1993 (JP) .  
5-243007 \* 9/1993 (JP) .  
7-29704 \* 1/1995 (JP) .  
9-0117609 6/1995 (JP) .

\* cited by examiner

*Primary Examiner*—Michael L. Gellner

*Assistant Examiner*—Kyung S. Lee

(74) *Attorney, Agent, or Firm*—Majestic, Parsons, Siebert & Hsue P.C.

(57) **ABSTRACT**

A chip thermistor has a pair of outer electrodes opposite each other with a specified distance in between on one of the surfaces of a thermistor element and an inner electrode extending inside the thermistor element so as to overlap these outer electrodes in the direction perpendicular to the surface on which the outer electrodes are formed. An electrically insulating layer is preferably formed on the same surface as and between the pair of outer electrodes. Each of the outer electrodes may be formed with two or more layers, the outermost of the layers being of gold.

**8 Claims, 4 Drawing Sheets**





FIG. 1



FIG. 2

**FIG.\_3A****FIG.\_3B****FIG.\_3C****FIG.\_3D****FIG.\_3E**

**FIG. 4****FIG. 5****FIG. 6****FIG. 7**



**FIG. 8A**  
(PRIOR ART)



**FIG. 8B**  
(PRIOR ART)



**FIG. 8C**  
(PRIOR ART)



**FIG. 9**  
(PRIOR ART)

## CHIP THERMISTORS

## BACKGROUND OF THE INVENTION

This invention relates to chip thermistors of the type which are commonly used for the protection of an electronic circuit or as a temperature-detecting sensor and, more particularly, to chip thermistors having electrodes formed overlappingly both on an outer surface of and inside a thermistor element.

The demand to be surface-mountable directly to a circuit board is just as strong on thermistors as on other kinds of electronic components. For this reason, many kinds of thermistors in the form of a chip (or chip thermistors) have been considered. FIG. 8A shows an example of prior art chip thermistor 61 having outer electrodes 63 and 64 formed at both end parts of a thermistor element 62. Each of the outer electrodes 63 and 64 is formed on one of the end surfaces and reaches the four side surfaces adjacent thereto such that the chip thermistor 61 can be surface-mounted, say, by soldering to electrode lands on a printed circuit board.

Inside the thermistor element 62, there may be inner electrodes 65, 66 and 67 each electrically connected to one of the outer electrodes 63 and 64, as shown in FIG. 8B, such that the resistance between the outer electrodes 63 and 64 is determined not only by the specific resistance (or the resistivity) of the thermistor element 62 but also the overlapping areas of the inner electrodes 65-67.

FIG. 8C shows another chip thermistor 68 of a kind having no inner electrodes inside its thermistor element 62. In this case, the resistance between the outer electrodes 63 and 64 is determined by the distance therebetween and the specific resistivity of the thermistor element 62.

FIG. 9 shows still another prior art chip thermistor 71 characterized as having outer electrodes 73 and 74 formed opposite each other on the upper surface of a thermistor element 72 of a semiconductor ceramic material such that they are separated by a specified distance D. In this example, the resistance is adjusted by the distance D of separation between the outer electrodes 73 and 74. Thus, this distance D must be changed for each type or lot of thermistors to be mass-produced, corresponding to the desired resistance. If the desired resistance value is very small, in particular, the distance of separation D must accordingly be made small, but if this distance D is made too small, the two outer electrodes 73 and 74 may contact each other. Since the rate of change in resistance per unit change in distance D becomes large as D is made smaller, it becomes difficult to control the resistance value and hence the variation in the resistance values of the obtained products also becomes large.

With prior art chip thermistors of the types shown in FIGS. 8A, 8B and 8C at 61 and 68, the variation  $3\sigma/x$  (where  $\sigma$  is the standard deviation and  $x$  is the average) in the resistance values is fairly large, being about 4-10%. Thus, there has been a strong demand to reduce this variation, say, to within about  $\pm 1\%$ , but it has been very difficult to respond to this demand. Another problem of this type of prior art chip thermistors was that a fillet is likely to be formed by a solder while it extends upward as it is surface-mounted, say, onto a printed circuit board from the bottom sides 63a and 64a of the outer electrodes 63 and 64 because this would make a high-density mounting difficult. Because of their shape, furthermore, these bottom sides 63a and 64a of the outer electrodes 63 and 64 cannot easily be bonded by a so-called bump-bonding method which is frequently used for effecting a high-density mounting.

## SUMMARY OF THE INVENTION

It is therefore an object of this invention to provide an improved type of chip thermistors of which the variation in the resistance values can be reduced.

It is another object of this invention to provide such chip thermistors which can be surface-mounted at a high density, allowing the use of a bump-bonding method.

A chip thermistor embodying this invention, with which the above and other objects can be accomplished, may be characterized as having a pair of outer electrodes formed opposite each other with a specified distance therebetween on one of the surfaces of a thermistor element and an inner electrode extending inside the thermistor element so as to overlap with these outer electrodes in the direction perpendicular to the surface on which the outer electrodes are formed. According to a preferred embodiment of the invention, an electrically insulating layer is disposed on the same surface as and between the pair of outer electrodes. Each of the outer electrodes may be formed with two or more layers, the outermost of the layers being of gold. The resistance value of such a chip thermistor can be adjusted by abrading at least a portion of the edges of the thermistor element together with portions of the outer electrodes.

## BRIEF DESCRIPTION OF THE DRAWINGS

The accompanying drawings, which are incorporated in and form a part of this specification, illustrate embodiments of the invention and, together with the description, serve to explain the principles of the invention. In the drawings:

FIG. 1 is a schematic diagonal view of a chip thermistor embodying this invention;

FIG. 2 is an equivalent circuit diagram of the chip thermistor of FIG. 1;

FIGS. 3A, 3B, 3C, 3D and 3E (together referred to as FIG. 3) are drawings for showing a method of producing chip thermistors as shown in FIG. 1;

FIG. 4 is a sectional view of a chip thermistor of which the resistance value has been adjusted by a method of this invention;

FIG. 5 is a sectional view of another chip thermistor embodying this invention;

FIG. 6 is a sectional view of a portion of an outer electrode structured differently according to this invention;

FIG. 7 is a sectional view of still another chip thermistor embodying this invention;

FIG. 8A is a diagonal view of a prior art chip thermistor, FIG. 8B is its sectional view, and FIG. 8C is a sectional view of another prior art chip thermistor; and

FIG. 9 is a diagonal view of still another prior art chip thermistor.

Throughout herein, like or equivalent components are indicated by the same numerals even where they are components of different devices and may not necessarily be described repetitiously.

## DETAILED DESCRIPTION OF THE INVENTION

FIG. 1 shows a chip thermistor 1 embodying this invention, having a rectangular planar thermistor element 2 which may comprise a semiconductor ceramic material with a positive or negative temperature coefficient. A pair of outer electrodes 3 and 4 is formed on the upper surface of the thermistor element 2, separated from each other with a

specified distance (herein referred to as "the gap") between their inner end edges oppositely facing each other and without covering the side surfaces of the planar thermistor element 2. Each of these outer electrodes 3 and 4 has a solder layer 3b or 4b of Au formed on top of an Ag—Pd layer 3a or 4a obtained by applying and firing an Ag—Pd paste. Their outer edges reach end surfaces 2a and 2b of the thermistor element 2, respectively. An electrically insulating layer 5 is formed directly on a center portion of the upper surface of the thermistor element 2 by burning a glass paste. As shown in FIG. 1, the inner end edges of the outer electrodes 3 and 4 reach the upper surface of the insulating layer 5. The invention does not limit the kind of glass paste which is used for forming the insulating layer 5.

Examples of glass paste which may be used for the purpose of this invention include those having lead borosilicate glass, zinc borosilicate glass, Bi borosilicate glass or Pb—Zn—Bi borosilicate glass as the main component. Alternatively, a synthetic resin such as polyimide resin, phenol resin or vinyl resin, synthetic rubber such as fluorine rubber, natural rubber or a material having an appropriate filler such as silica dispersed within such a resin or rubber material may be used for forming the insulating layer 5. In this case, however, the inner end edge parts of the outer electrodes 3 and 4 are formed so as to be under the lower surface of the insulator layer 5 because the insulating layer 5 is formed after the two outer electrodes 3 and 4 are formed by a burning process.

An inner electrode 6 is inside the thermistor element 2, serving not contacting the outer electrodes 3 and 4 and as a third electrode extending so as to overlap the outer electrodes 2 and 3 in the direction perpendicular to the surface on which the outer electrodes 2 and 3 are formed. The (third) inner electrode 6 may be formed by applying an electrode-forming paste by a printing process and carrying out a burning process simultaneously as the thermistor element 2 is produced.

The chip thermistor 1 thus formed can be surface-mounted, say, to a printed circuit board by connecting the outer electrodes 3 and 4 to electrode lands on the circuit board. Since each of the outer electrodes 3 and 4 is formed so as to have a flat smooth surface on the same surface of the thermistor element 2, a bump-bonding method can be used easily for the connection of the outer electrodes 3 and 4 to the circuit board.

The resistance characteristic of the chip thermistor 1 is critically dependent on the areas of the outer electrodes 3 and 4, the distance of separation therebetween and the thickness of the thermistor element 2. The chip thermistor 1 as described above may be considered to have the circuit structure as shown by an equivalent circuit diagram of FIG. 2, having a first resistance  $r_1$  between the first and second outer electrodes 3 and 4 connected in parallel with the series connection of a second resistance  $r_2$  between the electrodes 3 and 6 and the third resistance  $r_3$  between the electrodes 4 and 6.

Not only are chip thermistors embodying this invention easier to surface-mount than conventional chip thermistors, as described above, but the variation in their resistance values can be effectively reduced. This comes about because of the way the chip thermistors as described above can be produced. A method of producing chip thermistors as described above will be explained next with reference to FIG. 3.

For producing chip thermistors as shown in FIG. 1, a rectangular mother thermistor wafer 2A having inner elec-

trodes 6 already formed inside as shown in FIG. 3A is prepared. Next, a glass paste is applied by a screen printing process on mutually parallel areas on the thermistor wafer 2A, and the insulating layers 5A for the chip thermistors 1 are formed by a burning process. As shown in FIG. 3B, these insulating layers 5A are formed on the surface of the thermistor wafer 2A so as to extend from one of its side edges (2A<sub>1</sub>) to the opposite side edge 2A<sub>2</sub>. Next, the upper surface of the thermistor wafer 2A is coated with an Ag—Pd paste 7 by printing, as shown in FIG. 3C, such that the side edges of each strip of the insulating layer 5 are covered by the paste 7. Next, heat is applied to subject the Ag—Pd paste 7 to a burning process so as to form Ag—Pd layers 7A. Next, solder layers 9 are formed on the Ag—Pd layers 7A by soldering with Au, as shown in FIG. 3D. Finally, a mother thermistor 1A, as shown in FIG. 3E, is obtained by dicing the thermistor wafer 2A parallel to the direction in which the insulating layers 5 extend (referred to as the X-direction, as shown in FIG. 3E) and along center lines in the direction of the width of each Ag—Pd layers 7A.

Thereafter, the resistance of the mother thermistor 1A is measured, the length to which it should be diced in order to obtain therefrom a chip thermistor having a specified target resistance value is determined on the basis of this measured resistance value, and the mother thermistor 1A is diced in the Y-direction (perpendicular to the X-direction, as shown also in FIG. 3E) along two lines Y<sub>1</sub> and Y<sub>2</sub> separated by an appropriate distance, thereby obtaining a chip thermistor 1 as shown in FIG. 1.

Since the resistance values of the individual chip thermistors thus produced are determined as they are produced from their mother thermistors by dicing, the variation in their resistance values can be effectively reduced. This is so firstly because the outer electrodes 3 and 4 are formed so as to reach the top end of the end surfaces 2a and 2b of the thermistor element 2 and the resistance of the mother thermistor 1A is determined according to the accuracy of dicing in the X-direction for obtaining the mother thermistor 1A as shown in FIG. 3E. Since the dicing can be carried out very accurately, the resistance value of the mother thermistor 1A can be very accurately controlled. Secondly, the separation between the lines Y<sub>1</sub> and Y<sub>2</sub> along which the mother thermistor 1A is diced is determined on the basis of the actually measured resistance value of the mother thermistor 1A. Since the dicing can be carried out very accurately, as explained above, chip thermistors 1 with very small variations in the resistance values can be obtained.

In summary, the outer electrodes 3 and 4 of the chip thermistor 1 are formed so as to extend to the top end of the end surfaces 2a and 2b of the rectangular thermistor element 2 and also to the side surfaces 2c and 2d such that its resistance value is determined by the dicing processes carried out both in the X-direction and in the Y-direction. Thus, the variation in the resistance due, for example, to the variation in the areas of electrodes formed by screen printing can be reduced according to the present invention.

The resistance value of the chip thermistor 1 according to this invention can be varied also by adjusting the position of the inner electrode 6 while keeping the thickness of the thermistor element 2 constant. Thus, when chip thermistors having different resistance values are produced by using thermistor elements of the same size, variations in the occurrence of chips and cracks caused by the polishing for the adjustment of resistance can also be reduced.

This invention also relates to a method of adjusting the resistance value of a chip thermistor, as described above and

produced as described above, by abrading at least a portion of an edge or edges of the thermistor element together with portions of the outer electrodes.

As a test of this invention, a chip thermistor as shown in FIG. 1 was subjected to a barrel polishing process by using abrading balls of diameters 3–5 mm and water to abrade its edge portions. Throughout herein, the expression “edge portions” will be used to indicate the portions of the generally planar rectangular thermistor element along all its edges. As the edge portions are thus abraded, the areas of the first and second outer electrodes 3 and 4 become smaller, and this is how the resistance value of the chip thermistor 1 can be adjusted. In other words, chip thermistors with a desired target resistance value can be easily obtained by a barrel polishing process and the yield can thus be improved.

FIG. 5 shows another chip thermistor 21 embodying this invention which is similar to the chip thermistor 1 described above with reference to FIG. 1 but is different therefrom in that its outer electrodes 23 and 24 each consist an Ag—Pd layer 23a or 24a and a solder layer 23b or 24b thereon such that inner edge parts of the Ag—Pd layers 23a and 24a facing each other are exposed and an electrically insulating layer 25 is formed not only over the area between the two outer electrodes 23 and 24 but also on the exposed inner edge parts of the Ag—Pd layers 23a and 23b so as to contact the inner edges of the solder layers 23b and 24b which face each other. Such a chip thermistor 21 may be produced firstly by forming the Ag—Pd layers 23a and 23b on a thermistor element 2, secondly by applying and burning a glass paste to form the insulating layer 25, and thirdly by forming the solder layers 23b and 24b. Alternatively, the solder layers 23b and 24b may be formed first on the respective Ag—Pd layers 23a and 24a as shown in FIG. 5, say, by using a mask, the insulating layer 25 being formed thereafter. FIG. 5 shows the edge portions of the thermistor element 2 rounded, indicating that its resistance value has been adjusted by the method described above with reference to FIG. 4.

Although outer electrodes having an Ag—Pd layer and a solder layer of Au have been described above, the layer structure described above for illustration is not intended to limit the scope of the invention. The materials and the structure of the outer electrodes are not intended to limit the scope of the invention. They may be of a single metallic material. Alternatively, a different combinations of metals may be used.

FIG. 6 shows an example of an outer electrode structured differently, having three metallic layers 31, 32 and 33 formed one on top of another on a thermistor element 2. These layers may be formed by any of commonly used methods for forming thin films such as burning an electrically conductive paste, sputtering, vapor deposition and soldering. The thickness of each of the layers 31, 32 and 33 may be varied appropriately. The present inventors have ascertained that chip thermistors as shown at 1 in FIG. 1 with small variations in their resistance values can be obtained by using any of the six combinations of metals shown in Table 1 to form the three metallic layers 31, 32 and 33 of their outer electrodes.

TABLE 1-continued

| Combination No. | Layer 31 | Layer 32 | Layer 33 |
|-----------------|----------|----------|----------|
| 5               | 3        | Ti       | Pt       |
|                 | 4        | NiCr     | Ag       |
|                 | 5        | Ag       | Ni       |
|                 | 6        | Ag       | Cr       |
|                 |          |          | Au       |

10 FIG. 7 shows still another chip thermistor 41 embodying this invention which is similar to the chip thermistor 1 or 21 described above but is different therefrom in that a protective layer 47 is formed on the bottom surface of the thermistor element 2. Because of the protective layer 47 on the bottom surface, it is mostly the edge portions around the upper surface of the thermistor element 2 that are rounded off when the resistance value of the chip thermistor 41 is adjusted.

15 The present inventors have had many chip thermistors of this kind produced by using thermistor elements 2 with width 0.5 mm, length 1.0 mm, thickness 0.3 mm and resistivity about 2 kΩcm and by varying the distance d between the top surface of the thermistor element 2 and the inner electrode 6 so as to vary their resistance values. The 20 resistance values  $R_{25}$  of these different kinds of chip thermistors 41 at 25° C. and their deviations  $R_{3CV}(3\sigma/x)$  are shown in Table 2. Table 2 proves clearly that chip thermistors with different resistance values can be obtained easily by varying the height of the inner electrode and also that the variations in the resistance values are extremely 25 small.

TABLE 2

| d (mm)  | $R_{25}$ (kΩ) | $R_{3CV}$ (%) |
|---------|---------------|---------------|
| 35 0.16 | 30.1          | 3.3           |
| 0.12    | 22.5          | 3.4           |
| 0.08    | 17.3          | 3.2           |

40 Chip thermistors embodying this invention have many advantages. Firstly, since the outer electrodes are formed opposite to each other on the same surface of the thermistor element, the chip thermistor can be easily surface-mounted to a printed circuit board. Secondly, since the outer electrodes have flat and smooth surface areas on the same 45 surface of the thermistor element, fillets are not formed outside the thermistor element at the time of the surface-mounting. Thus, chip thermistors of this invention can be surface-mounted not only at a high density but also by a 50 bump-bonding process. Thirdly, since the outer electrodes are formed opposite to each other with a specified distance therebetween on the same surface of the thermistor element, chip thermistors of this invention can be obtained by first 55 producing a mother thermistor and then by dicing this mother thermistor. Since the dicing can be carried out very accurately, the variation in their resistance values can be easily reduced. Fourthly, with the presence of an inner electrode overlapping the outer electrode in the direction 60 perpendicular to the surface on which the outer electrodes are formed, the overall resistance value of the chip thermistor can be reduced and the variation in the resistance values of produced chip thermistors can also be reduced. If an insulating layer is provided between the pair of outer electrodes, the stability of the surface resistance between the outer electrodes is improved. This comes about because the 65 insulating layer thus formed serves to protect the semiconductor ceramics of the thermistor element from environmental elements such as moisture and dust particles.

TABLE 1

| Combination No. | Layer 31 | Layer 32 | Layer 33 |
|-----------------|----------|----------|----------|
| 1               | NiCr     | NiCu     | Au       |
| 2               | Ti       | Pd       | Au       |

What is claimed is:

1. A chip thermistor comprising:
  - a thermistor element having a top surface;
  - a pair of outer electrodes disposed entirely on said top surface and opposite each other with a gap of a specified width therebetween on said top surface of said thermistor element; and
  - an inner electrode not connected to said outer electrodes and extending parallel to said top surface inside said thermistor element so as to overlap said pair of outer electrodes as seen perpendicularly to said top surface.
2. The chip thermistor of claim 1 further comprising an electrically insulating layer disposed on said top surface of said thermistor element between said pair of outer electrodes.
3. The chip thermistor of claim 2 wherein said outer electrodes each consists of two or more layers, the outermost of said layers being a gold layer.

4. The chip thermistor of claim 1 wherein said outer electrodes each consists of two or more layers, the outermost of said layers being a gold layer.

5. The chip thermistor of claim 1 wherein said thermistor element is planar and has side surfaces which are perpendicular to said top surface and are not covered by said outer electrodes.

10 6. The chip thermistor of claim 5 wherein said outer electrodes each consists of two or more layers, the outermost of said layers being a gold layer.

7. The chip thermistor of claim 5 wherein said inner electrode is externally exposed at said side surfaces.

15 8. The chip thermistor of claim 6 wherein said inner electrode is externally exposed at said side surfaces.

\* \* \* \* \*